



US010563312B2

(12) **United States Patent**  
**Alrobei et al.**

(10) **Patent No.:** **US 10,563,312 B2**  
(b5) **Date of Patent:** **Feb. 18, 2020**

(54) **PHOTOELECTROCHEMICAL CELLS**

(71) Applicants: **Hussein Alrobei**, Tampa, FL (US);  
**Manoj Kumar Ram**, Palm Harbor, FL (US)

(72) Inventors: **Hussein Alrobei**, Tampa, FL (US);  
**Manoj Kumar Ram**, Palm Harbor, FL (US)

(73) Assignee: **University of South Florida**, Tampa, FL (US)

(\*) Notice: Subject to any disclaimer, the term of this patent is extended or adjusted under 35 U.S.C. 154(b) by 0 days.

(21) Appl. No.: **16/030,625**

(22) Filed: **Jul. 9, 2018**

(65) **Prior Publication Data**

US 2019/0017184 A1 Jan. 17, 2019

**Related U.S. Application Data**

(60) Provisional application No. 62/531,004, filed on Jul. 11, 2017.

(51) **Int. Cl.**

**C25B 11/04** (2006.01)  
**C25B 1/04** (2006.01)  
**C25B 9/06** (2006.01)  
**C25B 1/00** (2006.01)

(52) **U.S. Cl.**

CPC ..... **C25B 11/0489** (2013.01); **C25B 1/003** (2013.01); **C25B 1/04** (2013.01); **C25B 9/06** (2013.01); **C25B 11/04** (2013.01); **C25B 11/0405** (2013.01); **C25B 11/0415** (2013.01); **C25B 11/0478** (2013.01)

(58) **Field of Classification Search**

CPC ..... C25B 1/003  
See application file for complete search history.

(56) **References Cited**

## U.S. PATENT DOCUMENTS

4,240,882 A \* 12/1980 Ang ..... C25B 1/003  
204/252  
4,366,215 A \* 12/1982 Coetzer ..... H01M 4/36  
205/57  
4,414,080 A \* 11/1983 Williams ..... C25B 1/003  
204/242  
4,437,954 A \* 3/1984 Sammells ..... B01J 19/122  
204/157.15  
4,492,743 A \* 1/1985 Howe ..... C25B 1/003  
136/255

(Continued)

## FOREIGN PATENT DOCUMENTS

|    |             |        |
|----|-------------|--------|
| CN | 103703166 A | 4/2014 |
| CN | 103974769 A | 8/2014 |

## OTHER PUBLICATIONS

Alrobei et al, A New Insight in the Physical and Photoelectrochemical Properties of Molybdenum Disulfide Alpha-Hematite Nanocomposite Films, American Journal of Analytical Chemistry, vol. 8, Aug. 2017, pp. 523-539 (Year: 2017).\*

(Continued)

Primary Examiner — Harry D Wilkins, III

(74) Attorney, Agent, or Firm — Thomas|Horstemeyer, LLP

(57) **ABSTRACT**

Photoelectrochemical cells including a cathode including alpha-hematite and a metal dichalcogenide, an anode including a conducting polymer, and an electrolyte.

**15 Claims, 27 Drawing Sheets**



(56)

## References Cited

## U.S. PATENT DOCUMENTS

|              |     |         |                |                          |
|--------------|-----|---------|----------------|--------------------------|
| 8,361,288    | B2  | 1/2013  | Reece et al.   |                          |
| 9,416,456    | B1* | 8/2016  | Ram            | C25B 1/003               |
| 9,735,306    | B2* | 8/2017  | Carter         | H01L 31/0264             |
| 2010/0133110 | A1* | 6/2010  | Nocera         | C25B 1/003<br>205/340    |
| 2010/0133111 | A1  | 6/2010  | Nocera et al.  |                          |
| 2012/0267234 | A1* | 10/2012 | Reece          | B01J 19/127<br>204/157.5 |
| 2014/0000697 | A1  | 1/2014  | Wang et al.    |                          |
| 2015/0340166 | A1* | 11/2015 | Ren            | H01G 9/2013<br>136/254   |
| 2016/0193595 | A1* | 7/2016  | Nagpal         | C25B 3/04<br>502/215     |
| 2016/0194768 | A1  | 7/2016  | Toroker et al. |                          |

## OTHER PUBLICATIONS

- Zhang et al, Structural evolution and characteristics of the phase transformations between alpha-Fe2O3, Fe3O4, and gamma-Fe2O3 nanoparticles under reducing and oxidizing atmospheres, *CrystEngComm*, vol. 15, Aug. 2013, pp. 8166-8172 (Year: 2013).\*
- Ahn et al, MoSx supported hematite with enhanced photoelectrochemical performance, *Journal of Materials Chemistry A*, vol. 3, Oct. 2015, pp. 21444-21450 (Year: 2015).\*
- Ram et al, Novel Nano-hybrid Structured Regioregular Polyhexylthiophene Blend Films for Photoelectrochemical Energy Applications, *The Journal of Physical Chemistry C*, vol. 115, No. 44, Sep. 2011, pp. 21987-21995 (Year: 2011).\*
- Sivula et al, Solar Water Splitting: Progress Using Hematite (alpha-Fe2O3) Photoelectrodes, *ChemSusChem*, vol. 4, No. 4, Apr. 2011, pp. 432-449 (Year: 2011).\*
- Sun et al, MoS2 and graphene as dual, cocatalysts for enhanced visible light photocatalytic activity of Fe2O3, *Journal of Sol-Gel Science and Technology*, vol. 80, No. 3, Aug. 2016 (first online), pp. 719-727 (Year: 2016).\*
- Xiang et al, Synergetic Effect of MoS2 and Graphene as Cocatalysts for Enhanced Photocatalytic H2 Production Acitivity of TiO2 Nanoparticles, *Journal of the American Chemical Society*, vol. 134, No. 15, Mar. 2012, pp. 6575-6578 (Year: 2012).\*
- Ahn et al., "Nanoporous Hematite Structures to Overcome Short Diffusion Lengths in Water Splitting," *Journal of Materials Chemistry A*, 2014, 2, 19999-20003.
- Alrobei et al., "Aluminum Doped  $\alpha$ -Hematite for Photoelectrochemical Applications," Research Day 2015 at USF College of Engineering, 2015. Tampa, Florida, USA.
- Alrobei et al., "Aluminum- $\alpha$ -Hematite Thin Films for Photoelectrochemical Applications," *Surface Review and Letters*, 2017, 1950031.
- Alrobei et al., "Doped  $\alpha$ -hematite with Molybdenum Sulfides MoS<sub>2</sub> for photoelectrochemical applications," 9th Annual College of Engineering Research Day, 2016. Tampa, FL, USA.
- Alrobei et al., "p-n Based Photoelectrochemical Device for Water Splitting Application Alpha-Hematite ( $\alpha$ -Fe<sub>2</sub>O<sub>3</sub>)-Titanium Dioxide (TiO<sub>2</sub>) as N-Electrode & Polyhexylthiophene (RRPHTH)-Nanodiamond (ND) as P-Electrode," *MRS Advances*, 2017.
- Alrobei et al., "Molybdenum disulfide Doped  $\alpha$ -Hematite for Photoelectrochemical Applications," Poster presented at 9th Annual College of Engineering Research Day, 2016. Tampa, FL, USA.
- Basnayaka et al., "Photovoltaic properties of multi walled carbon nanotubes-poly(3-octathiophene) conducting polymer blends structures," *MRS Proceedings*, 2013, Cambridge University Press, Cambridge, 139-144.
- Bassi et al., "Iron Based Photoanodes for Solar Fuel Production," *Physical Chemistry Chemical Physics*, 2014, 16, 11834-11842.
- Bonde et al., "Hydrogen Evolution on Nano-Particulate Transition Metal Sulfides," *Faraday Discussions*, 2009, 140, 219-231.
- Cesar et al., "Translucent thin film Fe<sub>2</sub>O<sub>3</sub> photoanodes for efficient water splitting by sunlight: nanostructure-directing effect of Si-doping," *Journal of the American Chemical Society*, 2006, 128(14): 4582-4583.
- Chemelewski et al., "Bandgap engineering of Fe<sub>2</sub>O<sub>3</sub> with Cr—application to photoelectrochemical oxidation," *Physical Chemistry Chemical Physics*, 2016, 18(3): 1644-1648.
- Chen et al., "Core-Shell MoO<sub>3</sub>—MoS<sub>2</sub> Nanowires for Hydrogen Evolution: A Functional Design for Electrocatalytic Materials," *Nano Letters*, 2011, 11, 4168-4175.
- Chirita et al., " $\text{Fe}_2\text{O}_3$ —nanoparticles, physical properties and their photochemical and photoelectrochemical applications," *Chem. Bull.*, 2009, 54(68): 1-8.
- Choi et al., "High-detectivity multilayer MoS<sub>2</sub> phototransistors with spectral response from ultraviolet to infrared," *Advanced materials*, 2012, 24(43): 5832-5836.
- Desai et al., "FT-IR, XPS and PEC Characterization of Spray Deposited Hematite Thin Films," *Applied Surface Science*, 2005, 252, 1870-1875.
- Ding et al., "Efficient Photoelectrochemical Hydrogen Generation using Heterostructures of Si and Chemically Exfoliated Metallic MoS<sub>2</sub>," *Journal of the American Chemical Society*, 2014, 136, 8504-8507.
- Du et al., "Hematite-Based Water Splitting with Low Turn-On Voltages," *Angewandte Chemie International Edition*, 2013, 52, 12924-12927.
- Duret et al., "Visible light-induced water oxidation on mesoscopic  $\alpha$ -Fe<sub>2</sub>O<sub>3</sub> films made by ultrasonic spray pyrolysis," *The Journal of Physical Chemistry B*, 2005, 109(36): 17184-17191.
- Gao et al., "Ferromagnetism in Freestanding MoS<sub>2</sub> Nanosheets," *Nanoscale Research Letters*, 2013, 8: 129, 8 pages.
- Giambrone et al., "Comparative Photoelectrochemical Studies of Regioregular Polyhexylthiophene with Microdiamond, Nanodiamond and Hexagonal Boron Nitride Hybrid Films," *Thin Solid Films*, 2016, 615, 226-232.
- Hahn et al., "Reactive ballistic deposition of  $\alpha$ -Fe<sub>2</sub>O<sub>3</sub> thin films for photoelectrochemical water oxidation," *ACS nano*, 2010, 4(4): 1977-1986.
- Han et al., "One-Step Hydrothermal Synthesis of 2D Hexagonal Nanoplates of  $\alpha$ -Fe<sub>2</sub>O<sub>3</sub>/Graphene Composites with Enhanced Photocatalytic Activity," *Advanced Functional Materials*, 2014, 24(36): 5719-5727.
- He et al., "Fabrication of Flexible MoS<sub>2</sub> Thin-Film Transistor Arrays for Practical Gas-Sensing Applications" *Small*, 2012, 8(19): 2994-2999.
- Hiralal et al., "Nanostructured hematite photoelectrochemical electrodes prepared by the low temperature thermal oxidation of iron," *Solar Energy Materials and Solar Cells*, 2011, 95(7): 1819-1825.
- Hisatomi et al., "Enhancement in the Performance of Ultrathin Hematite Photoanode for Water Splitting by an Oxide Underlayer," *Advanced Materials*, 2012, 24, 2699-2702.
- Hisatomi et al., "Recent advances in semiconductors for photocatalytic and photoelectrochemical water splitting," *Chemical Society Reviews*, 2014, 43(22): 7520-7535.
- Hu et al., "Pt-doped  $\alpha$ -Fe<sub>2</sub>O<sub>3</sub> thin films active for photoelectrochemical water splitting," *Chemistry of Materials*, 2008, 20(12): 3803-3805.
- Jorand Sartoretti et al., "Photoelectrochemical oxidation of water at transparent ferric oxide film electrodes," *The Journal of Physical Chemistry B*, 2005, 109(28): 13685-13692.
- Kay et al., "New benchmark for water photooxidation by nanostructured  $\alpha$ -Fe2O3 films," *Journal of the American Chemical Society*, 2006, 128(49): 15714-15721.
- Kennedy et al., "Photooxidation of water at  $\alpha$ -Fe<sub>2</sub>O<sub>3</sub> electrodes," *Journal of the Electrochemical Society*, 1978, 125(5): 709-714.
- Kibsgaard et al., "Engineering the Surface Structure of MoS<sub>2</sub> to Preferentially Expose Active Edge Sites for Electrocatalysis," *Nature Materials*, 2012, 11, 963-969.
- Kim et al., "Single-Crystalline, Wormlike Hematite Photoanodes for Efficient Solar Water Splitting," *Scientific reports*, 2013, 3: 2681, 8 pages.
- Kleiman-Shwarscstein et al., "Electrodeposited Aluminum-Doped  $\alpha$ -Fe<sub>2</sub>O<sub>3</sub> Photoelectrodes: Experiment and Theory," *Chemistry of Materials*, 22, 2009, 510-517.
- Kleiman-Shwarscstein et al., "Electrodeposition of  $\alpha$ -Fe<sub>2</sub>O<sub>3</sub> doped with Mo or Cr as photoanodes for photocatalytic water splitting," *The Journal of Physical Chemistry C*, 2008, 112(40): 15900-15907.

(56)

## References Cited

## OTHER PUBLICATIONS

- Knen et al., "On the Improvement of PEC Activity of Hematite Thin Films Deposited by High-Power Pulsed Magnetron Sputtering Method," *Applied Catalysis B: Environmental*, 2015, 165, 344-350.
- Koutsoukos et al., "Protein adsorption on hematite ( $\alpha$ -Fe<sub>2</sub>O<sub>3</sub>) surfaces," *Journal of colloid and interface science*, 1983, 95(2): 385-397.
- Kumari et al., "Characterization of Zn-Doped Hematite Thin Films for Photoelectrochemical Splitting of Water," *Current Science*, 2006, 91, 1062-1064.
- Lee et al., "MoS<sub>2</sub> nanosheet phototransistors with thickness-modulated optical energy gap," *Nano letters*, 2012, 12(7): 3695-3700.
- Li et al., "Fabrication of single-and multilayer MoS<sub>2</sub> film-based field-effect transistors for sensing NO at room temperature" *Small*, 2012, 8(1): 63-67.
- Li et al., "MoS<sub>2</sub> nanoparticles grown on graphene: an advanced catalyst for the hydrogen evolution reaction," *Journal of the American Chemical Society*, 2011, 133(19): 7296-7299.
- Lin et al., "Nanonet-based hematite heteronanostructures for efficient solar water splitting," *Journal of the American Chemical Society*, 2011, 133(8): 2398-2401.
- Liu et al., "MoS<sub>2</sub>/CdS Heterojunction with High Photoelectrochemical Activity for H<sub>2</sub> Evolution under Visible Light: The Role of MoS<sub>2</sub>," *The Journal of Physical Chemistry C*, 2013, 117(25): 12949-12957.
- Liu et al., "Photoelectrochemical properties of Ni-doped Fe<sub>2</sub>O<sub>3</sub> thin films prepared by electrodeposition," *Electrochimica Acta*, 2012, 59: 121-127.
- Mehraj et al., "A highly efficient visible-light-driven novel pn junction Fe<sub>2</sub>O<sub>3</sub>/BiOI photocatalyst: Surface decoration of BiOI nanosheets with Fe2O3 nanoparticles," *Applied Surface Science*, 2016, 387: 642-651.
- Melero et al., "Nanocomposite Fe<sub>2</sub>O<sub>3</sub>/SBA-15: An efficient and stable catalyst for the catalytic wet peroxidation of phenolic aqueous solutions," *Chemical Engineering Journal*, 2007, 131(1-3): 245-256.
- Meng et al., "Photocatalytic Water Oxidation by Hematite/Reduced Graphene Oxide Composites," *ACS Catalysis*, 2013, 3, 746-751.
- Meng et al., "Solar hydrogen generation by nanoscale p-n junction of p-type molybdenum disulfide/n-type nitrogen-doped reduced graphene oxide," *Journal of the American Chemical Society*, 2013, 135(28): 10286-10289.
- Miao et al., "Surface plasmon-enhanced photodetection in few layer MoS<sub>2</sub> phototransistors with Au nanostructure arrays," *Small*, 2015, 11(20): 2392-2398.
- Mohapatra et al., "Water photooxidation by smooth and ultrathin  $\alpha$ -Fe<sub>2</sub>O<sub>3</sub> nanotube arrays," *Chemistry of Materials*, 2009, 21(14): 3048-3055.
- Ram et al., "A New Insight in the Physical and Photoelectrochemical Properties of Molybdenum Disulfide Alpha-Hematite Nanocomposite Films," *American Journal of Analytical Chemistry*, 2017, 8(08): 523-539.
- Ram et al., "Performance of electrochromic cells of polyaniline in polymeric electrolytes," *Journal of materials science letters*, 1994, 13(20): p. 1490-1493.
- Ram et al., "The Electrochromic Response of Polyaniline and Its Copolymeric Systems," *Thin Solid Films*, 1997, 303, 27-33.
- Sahoo et al., "Characterization of  $\gamma$ -and  $\alpha$ -Fe<sub>2</sub>O<sub>3</sub> nano powders synthesized by emulsion precipitation-calcination route and rheological behaviour of  $\alpha$ -Fe<sub>2</sub>O<sub>3</sub>," *International Journal of Engineering, Science and Technology*, 2010, 2(8): 118-126.
- Saremi-Yarahmadi et al., "Nanostructured  $\alpha$ -Fe<sub>2</sub>O<sub>3</sub> electrodes for solar driven water splitting: effect of doping agents on preparation and performance," *The Journal of Physical Chemistry C*, 2009, 113(12): 4768-4778.
- Satsangi et al., "Nanostructured Hematite for Photoelectrochemical Generation of Hydrogen," *International Journal of Hydrogen Energy*, 2008, 33, 312-318.
- Shinde et al., "Physical properties of hematite  $\alpha$ -Fe<sub>2</sub>O<sub>3</sub> thin films: application to photoelectrochemical solar cells," *Journal of Semiconductors*, 2011, 32(1): 013001, 8 pages.
- Srivastava, "Synthesis and Characterization of Iron Oxide Nanoparticle from FeCl<sub>3</sub> by Using Polyvinyl Alcohol," *International Journal of Physical and Social Sciences*, 2012, 2, 161-184.
- Sun et al., "Observation of a Burstein-Moss shift in rhenium-doped MoS<sub>2</sub> nanoparticles," *ACS nano*, 2013, 7(4): 3506-3511.
- Tamirat et al., "Using Hematite for Photoelectrochemical Water Splitting: A Review of Current Progress and Challenges," *Nanoscale Horizons*, 2016, 1, 243-267.
- Thurston et al., "Photooxidation of Organic Chemicals Catalyzed by Nanoscale MoS<sub>2</sub>," *The Journal of Physical Chemistry B*, 1999, 103, 11-17.
- Van de Krol et al., "Solar hydrogen production with nanostructured metal oxides," *Journal of Materials Chemistry*, 2008, 18(20): 2311-2320.
- Wheeler et al., "Nanostructured hematite: synthesis, characterization, charge carrier dynamics, and photoelectrochemical properties," *Energy & Environmental Science*, 2012, 5(5): 6682-6702.
- Woo et al., "Sol-Gel Mediated Synthesis of Fe<sub>2</sub>O<sub>3</sub> Nanorods," *Advanced Materials*, 2003, 15, 1761-1764.
- Wu et al., "Electrochemically reduced single-layer MoS<sub>2</sub> nanosheets: Characterization, properties, and sensing applications," *Small*, 2012, 8(14): 2264-2270.
- Xiang et al., "Synergistic effect of MoS<sub>2</sub> and graphene as cocatalysts for enhanced photocatalytic H<sub>2</sub> production activity of TiO<sub>2</sub> nanoparticles," *Journal of the American Chemical Society*, 2012, 134(15): 6575-6578.
- Yang et al., "High Efficient Photo-Fenton Catalyst of  $\alpha$ -Fe<sub>2</sub>O<sub>3</sub>/MoS<sub>2</sub> Hierarchical Nanoheterostructures: Reutilization for Supercapacitors," *Scientific Reports*, 2016, 6, Article No. 31591, 12 pages.
- Ye et al., "Fabrication and Enhanced Photoelectrochemical Performance of MoS<sub>2</sub>/S-Doped G-C<sub>3</sub>N<sub>4</sub> Heterojunction Film," *ACS Applied Materials & Interfaces*, 2016, 8, 5280-5289.
- Yin et al., "Single-layer MoS<sub>2</sub> phototransistors," *ACS nano*, 2011, 6(1): 74-80.
- Yoon et al., "Hematite-Based Photoelectrochemical Water Splitting Supported by Inverse Opal Structures of Graphene," *ACS Applied Materials & Interfaces*, 2014, 6, 22634-22639.
- Zhang et al., "Synthesis of S-rich flower-like Fe<sub>2</sub>O<sub>3</sub>-MoS<sub>2</sub> for Cr(VI) removal," *Separation Science and Technology*, 2016, 51(11): 1779-1786.

\* cited by examiner



FIG. 1

FIG. 2A



FIG. 2B



FIG. 2C



FIG. 2D



FIG. 2E



FIG. 2F



FIG. 3



FIG. 4



FIG. 5



FIG. 6A



FIG. 6B



FIG. 7



FIG. 8



FIG. 9

FIG. 10A



FIG. 10B



FIG. 11A



FIG. 11B





FIG. 12



FIG. 13



FIG. 14A  
FIG. 14B



FIG. 14C



FIG. 15A



FIG. 15B



FIG. 15C



FIG. 16B



FIG. 16A



FIG. 17A



FIG. 17B



FIG. 17C



FIG. 18



FIG. 19



FIG. 20



FIG. 21



FIG. 22



FIG. 23A

FIG. 23B



ND-RRPHTh



FIG. 24



FIG. 25



FIG. 26

## PHOTOELECTROCHEMICAL CELLS

## CROSS-REFERENCE TO RELATED APPLICATIONS

This application claims the benefit of and priority to U.S. Provisional Patent Application No. 62/531,004, filed on Jul. 11, 2017, the entire contents of which are fully incorporated herein by reference.

## BACKGROUND OF THE INVENTION

Photoelectrochemical cells have been used to convert solar energy to hydrogen gas by splitting water into hydrogen and oxygen, hence offering the possibility of clean and renewable energy. Many photoelectrochemical cells have used titanium dioxide ( $TiO_2$ ), but the large band gap of  $TiO_2$  (about 3.1-3.3 eV) impedes the absorption of visible light and limits the solar-to-hydrogen efficiency to about 2.2%. So, it is necessary to use other materials that have a smaller band gap and can more efficiently harvest energy from sunlight.

There are many semiconductor materials with a lower band gap than  $TiO_2$ , such as iron oxide ( $Fe_2O_3$ ), bismuth vanadium oxide ( $BiVO_4$ ), tungsten oxide ( $WO_3$ ) and tantalum nitride ( $Ta_3N_5$ ), for example. Alpha ( $\alpha$ )-hematite, in particular, has a solar-to-hydrogen conversion efficiency of about 16%. Additionally,  $\alpha$ - $Fe_2O_3$  has a low bandgap (2.1-2.2 eV), low cost, high chemical stability, nontoxicity, and natural abundance. It has several drawbacks as well, however, such as a relatively short hole diffusion length, low conductivity, shorter lifetime of photoexcitation, and deprived reaction kinetics of oxygen evolution. Some have tried doping with certain metals, such as titanium (Ti), molybdenum (Mo), aluminum (Al), zinc (Zn), platinum (Pt), and silicon (Si), for example, to improve the PEC performance of  $\alpha$ - $Fe_2O_3$ .

## SUMMARY OF THE INVENTION

The present invention relates to photoelectrochemical cells (PEC). More particularly, it relates to photoelectrochemical cells including  $\alpha$ - $Fe_2O_3$  and molybdenum disulfide ( $MoS_2$ ).

In one embodiment, the invention provides a photoelectrochemical cell, which includes a cathode that includes  $\alpha$ - $Fe_2O_3$  and a metal dichalcogenide, an anode that includes a conducting polymer, and an electrolyte.

In another embodiment, the invention provides a method of producing a photoelectrochemical cell, which includes a cathode that includes  $\alpha$ - $Fe_2O_3$  and a metal dichalcogenide, an anode that includes a conducting polymer, and an electrolyte.

In yet another embodiment, the invention provides a method of generating hydrogen from water with a photoelectrochemical cell, which includes a cathode that includes  $\alpha$ - $Fe_2O_3$  and a metal dichalcogenide, an anode that includes a conducting polymer, and an electrolyte.

Other aspects of the invention will become apparent by consideration of the detailed description and accompanying drawings.

## BRIEF DESCRIPTION OF THE DRAWINGS

FIG. 1 shows the chemical structure and photographs of  $MoS_2$ - $\alpha$ - $Fe_2O_3$  nanomaterial.

FIGS. 2A-2F show UV-visible absorption spectra of  $MoS_2$  with  $\alpha$ - $Fe_2O_3$  nanocomposite.

FIG. 3 shows powder X-ray diffraction patterns of  $MoS_2$  with  $\alpha$ - $Fe_2O_3$  nanocomposite.

FIG. 4 shows FTIR spectra of  $MoS_2$  with  $\alpha$ -hematite nanocomposite. Each curve  $MoS_2$  doping with  $Fe_2O_3$  is given as: Curve 1=5%  $MoS_2$ , Curve 2=0.2%  $MoS_2$ - $Fe_2O_3$ , Curve 3=2%  $MoS_2$ - $Fe_2O_3$ , Curve 4=1%  $MoS_2$ - $Fe_2O_3$ , Curve 5=0.5%  $MoS_2$ - $Fe_2O_3$  and Curve 6=0.1%  $MoS_2$ - $Fe_2O_3$ .

FIG. 5 shows scanning electron micrographs (SEM) of  $MoS_2$  with  $\alpha$ - $Fe_2O_3$  nanocomposite.

FIGS. 6A and 6B show Raman spectra of  $MoS_2$ - $\alpha$ - $Fe_2O_3$  film sample and ITO substrate as various percentage of  $MoS_2$ .

FIG. 7 shows the particle size measurement of  $MoS_2$ - $\alpha$ - $Fe_2O_3$  nanocomposite materials as a function of  $MoS_2$  dopant.

FIG. 8 shows cyclic voltammetry of about 1%  $MoS_2$  with  $Fe_2O_3$  nanocomposite without light in about 1 M NaOH.

FIG. 9 shows cyclic voltammetry of about 1%  $MoS_2$  with  $Fe_2O_3$  nanocomposite with light in about 1 M NaOH.

FIGS. 10A and 10B show the chronoamperometry photocurrent plots with  $t(s)^{-1/2}$  for oxidation and reduction processes for  $MoS_2$ - $\alpha$ - $Fe_2O_3$  film.

FIGS. 11A and 11B show Nyquist plots of  $MoS_2$ - $\alpha$ - $Fe_2O_3$  film in 1 M HCl in photoelectrochemical cell without (FIG. 11A) and with (FIG. 11B) light irradiation.

FIG. 12 shows half sweep potential with and without light for Al doped- $\alpha$ - $Fe_2O_3$  and for  $MoS_2$ - $\alpha$ - $Fe_2O_3$  film.

FIG. 13 shows a schematic of hydrogen production using  $MoS_2$ -composite  $\alpha$ - $Fe_2O_3$  photocatalyst in about 1 M NaOH.

FIGS. 14A-14C show scanning electron micrographs (SEM) of  $Fe_2O_3$  (FIG. 14A),  $Fe_2O_3$ +0.1%  $MoS_2$  (FIG. 14B), and regioregular polyhexylthiophene (RRPHTH)+nanodiamond (ND) (FIG. 14C).

FIGS. 15A-15C show FTIR spectra of  $Fe_2O_3$  (FIG. 15A),  $Fe_2O_3$ +0.1%  $MoS_2$  (FIG. 15B), and RRPHTH+ND (FIG. 15C).

FIGS. 16A-16B show X-ray diffraction patterns of  $Fe_2O_3$  (FIG. 16A) and  $Fe_2O_3$ +0.1%  $MoS_2$  (FIG. 16B).

FIGS. 17A-17C show UV-vis absorption spectra of  $Fe_2O_3$  (FIG. 17A),  $Fe_2O_3$ +0.1%  $MoS_2$  (FIG. 17B), and RRPHTH+ND (FIG. 17C).

FIG. 18 shows a schematic of a water splitting application in p-type RRPHTH-ND and n-type  $MoS_2$ - $Fe_2O_3$  in water based electrolyte, in a photoelectrochemical cell under a photoexcitation and under potential.

FIG. 19 shows cyclic voltammetry of p-type RRPHTH-ND and n-type  $MoS_2$ - $Fe_2O_3$  in about 1 M NaOH based electrolyte, in a photochemical cell with and without light.

FIG. 20 shows current-transient data of p-type RRPHTH-ND and n-type 0.1%  $MoS_2$ - $Fe_2O_3$  electrodes in about 1 M NaOH based electrolyte, in a photoelectrochemical cell with and without light.

FIG. 21 shows current-transient data for a photoelectrochemical cell containing an RRPHTH-ND p-type electrode and about 0.1%, 0.2%, 1%, and 5%  $MoS_2$  in  $MoS_2$ - $Fe_2O_3$  n-type electrodes in about 1 M NaOH based electrolyte, with a light switch on and off at an applied potential of about 1500 mV.

FIG. 22 shows current-transient data for a photoelectrochemical cell containing an RRPHTH-ND p-type electrode and about 0.1%, 0.2%, 1%, and 5%  $MoS_2$  in  $MoS_2$ - $Fe_2O_3$

n-type electrodes in about 1 M NaOH based electrolyte, with a light switch on and off at an applied potential of about 2000 mV.

FIG. 23A shows a schematic of hydrogen production using MoS<sub>2</sub>-composite  $\alpha$ -Fe<sub>2</sub>O<sub>3</sub> as n-type and RRPHTH-ND as p-type photocatalyst in 1 M NaOH.

FIG. 23B shows the chemical structure of nanodiamond in a regioregular polyhexylthiophene blend structure.

FIG. 24 shows a schematic of a solid photoelectrochemical cell.

FIG. 25 shows current-transient data for a photoelectrochemical cell containing an RRPHTH-ND p-type electrode and about 1% MoS<sub>2</sub> in a MoS<sub>2</sub>—Fe<sub>2</sub>O<sub>3</sub> n-type electrode in about 1 M NaOH based electrolyte, with a light switch on and off at different applied potentials.

FIG. 26 shows current-transient data for a photoelectrochemical cell containing an RRPHTH-ND p-type electrode and a TiO<sub>2</sub>- $\alpha$ -Fe<sub>2</sub>O<sub>3</sub> n-type electrode in about 1 M NaOH based electrolyte, with a light switch on and off at an applied potential from about 0-2000 mV.

#### DETAILED DESCRIPTION

Before any embodiments of the invention are explained in detail, it is to be understood that the invention is not limited in its application to the details of construction and the arrangement of components set forth in the following description or illustrated in the following drawings. The invention is capable of other embodiments and of being practiced or of being carried out in various ways.

The terms “comprise(s),” “include(s),” “having,” “has,” “can,” “contain(s),” and variants thereof, as used herein, are intended to be open-ended transitional phrases, terms, or words that do not preclude the possibility of additional acts or structures. The singular forms “a,” “and,” and “the” include plural references unless the context clearly dictates otherwise. The present disclosure also contemplates other embodiments “comprising,” “consisting of,” and “consisting essentially of,” the embodiments or elements presented herein, whether explicitly set forth or not.

The conjunctive term “or” includes any and all combinations of one or more listed elements associated by the conjunctive term. For example, the phrase “an apparatus comprising A or B” may refer to an apparatus including A where B is not present, an apparatus including B where A is not present, or an apparatus where both A and B are present. The phrase “at least one of A, B, . . . and N” or “at least one of A, B, . . . N, or combinations thereof” are defined in the broadest sense to mean one or more elements selected from the group comprising A, B, . . . and N, that is to say, any combination of one or more elements A, B, . . . or N including any one element alone or in combination with one or more of the other elements, which may also include, in combination, additional elements not listed.

The modifier “about” used in connection with a quantity is inclusive of the stated value and has the meaning dictated by the context (for example, it includes at least the degree of error associated with the measurement of the particular quantity). The modifier “about” should also be considered as disclosing the range defined by the absolute values of the two endpoints. For example, the expression “from about 2 to about 4” also discloses the range “from 2 to 4”. The term “about” may refer to plus or minus 10% of the indicated number. For example, “about 10%” may indicate a range of 9% to 11%, and “about 1%” may mean from 0.9-1.1. Other

meanings of “about” may be apparent from the context, such as rounding off, so, for example “about 1” may also mean from 0.5 to 1.4.

For the recitation of numeric ranges herein, each intervening number there between with the same degree of precision is explicitly contemplated. For example, for the range of 6-9, the numbers 7 and 8 are contemplated in addition to 6 and 9, and for the range 6.0-7.0, the number 6.0, 6.1, 6.2, 6.3, 6.4, 6.5, 6.6, 6.7, 6.8, 6.9, and 7.0 are explicitly contemplated.

Unless otherwise defined, all technical and scientific terms used herein have the same meaning as commonly understood by one of ordinary skill in the art. In case of conflict, the present document, including definitions, will control. Preferred methods and materials are described below, although methods and materials similar or equivalent to those described herein can be used in practice or testing of the present invention. All publications, patent applications, patents and other references mentioned herein are incorporated by reference in their entirety. The materials, methods, and examples disclosed herein are illustrative only and not intended to be limiting.

#### 1. PHOTOCHEMICAL CELL

In one aspect, provided is a photoelectrochemical cell comprising:

- (a) a cathode comprising a-hematite and a metal dichalcogenide;
- (b) an anode comprising a conducting polymer; and
- (c) an electrolyte.

In some embodiments, the a-hematite includes a dopant. Suitable dopants include, but are not limited to platinum, tin, cobalt, zinc, palladium, titanium, chromium, rhodium, iridium, and combinations thereof.

Suitable metal dichalcogenides include, but are not limited to, molybdenum disulfide, tungsten disulfide, molybdenum diselenide, molybdenum telluride, tungsten selenide, and combinations thereof. In certain embodiments, the metal dichalcogenide is molybdenum disulfide (MoS<sub>2</sub>). The content of the metal dichalcogenide may range from about 0.1% to about 10% in a-hematite, including from about 0.1% to about 5%, from about 0.1% to about 1%, or from about 1% to about 5%. In certain embodiments, the content of the metal dichalcogenide is at a level of about 0.1%, about 0.2%, about 0.5%, about 1%, about 2%, or about 5% in  $\alpha$ -hematite. In some embodiments, the metal dichalcogenide is MoS<sub>2</sub> at a level of about 0.1%, about 0.2%, about 0.5%, about 1%, about 2%, or about 5% in  $\alpha$ -hematite.

Suitable conducting polymers include, but are not limited to polythiophenes, polyhexylthiophene, regioregular polyhexylthiophene, polyethylenedioxythiophene, polymethylthiophene, polydodcylthiophene, polycarbazole, poly(n-vinylcarbazole), substituted polyethylenedioxythiophenes, polydioxythiophene, polyaniline, n-poly(N-methyl aniline), poly(o-ethoxyaniline), poly(o-toluidine), poly(phenylene vinylene), and combinations thereof.

In some embodiments, the anode includes an electron acceptor. Suitable electron acceptors include, but are not limited to, diamond, nanodiamond, hexagonal boro-nitride (hBN), graphite, methyl [6, 6]-phenyl-C61-butrate (PCBM), 2,4,7-trinitro-9-fluorenone, copper-phthalocyanines, and combinations thereof.

Suitable electrolytes include, but are not limited to, aqueous electrolytes known in the art. In some embodiments, the electrolyte is a an aqueous electrolyte which comprises sodium hydroxide, potassium hydroxide, magnesium

hydroxide, lithium hydroxide, sodium chloride, potassium chloride, magnesium chloride, hydrochloric acid, sulfuric acid, nitric acid, acetic acid, butyric acid, lactic acid, oxalic acid, myristic acid, and/or perchloric acid.

In some embodiments, the electrolyte of the disclosed photoelectrochemical is in the form of a gel. For example, the electrolyte may be a gel comprising a polymer and an acid.

In some embodiments, the electrolyte is a gel comprising a polymer and an acid, in which the polymer is polyvinyl alcohol, poly(vinyl acetate), poly(vinyl alcohol co-vinyl acetate), poly(methyl methacrylate), poly(vinyl alcohol-co-ethylene ethylene), poly(vinyl butyral-co-vinyl alcohol-co-vinyl acetate), polyvinyl butyral, polyvinyl chloride, polystyrene, or combinations thereof. Suitable polymers for the gel form electrolyte may include others known in the art.

In some embodiments, the electrolyte is a gel comprising a polymer and an acid, in which the acid is acetic acid, propionic acid, hydrochloric acid, hydrofluoric acid, phosphoric acid, sulfuric acid, formic acid, benzoic acid, hydrofluoric acid, nitric acid, phosphoric acid, sulfuric acid, tungstosilicic acid hydrate, hydriodic acid, carboxylic acid, or combinations thereof. Suitable acids for the gel form electrolyte may include others known in the art.

In some embodiments, the cathode of the disclosed photoelectrochemical cell is a nanostructured film.

In some embodiments, the disclosed photoelectrochemical cell is capable of being stable, of being essentially free of photocorrosion, of preventing leakage of solvent, and/or of having low absorption of light.

The disclosed photoelectrochemical cell may produce a photocurrent. In some embodiments, the intensity of a photocurrent produced by the disclosed photoelectrochemical cell is dependent on the concentration of the electrolyte.

The disclosed photoelectrochemical cell may be capable of producing at least 10 times, at least 50 times, at least 100 times, or even at least 200 times difference in stable photocurrent at different applied potentials. In some embodiments, the disclosed photoelectrochemical cell is capable of producing at least a 100 times difference in stable photocurrent at different applied potentials.

## 2. METHODS

In another aspect, provided is a method of generating hydrogen from water, which comprises providing a photoelectrochemical cell as described herein.

In some embodiments, the photoelectrochemical cell used in the disclosed method comprises ND-RRPHTh blend film as a p-type electrode, MoS<sub>2</sub>- $\alpha$ -hematite as an n-type electrode, and an acidic or a basic solution.

In some embodiments, the disclosed method further comprises splitting water into hydrogen and oxygen by means of photocurrent from a p-n junction of the electrochemical cell.

The disclosed method of generating hydrogen from water may achieve a photocurrent. In some embodiments, the photocurrent obtained in the disclosed method is at a potential from about 0 V to about 2 V.

In another aspect, provided is a method of producing a photoelectrochemical cell as described herein, which comprises:

- Depositing about 1% MoS<sub>2</sub>- $\alpha$ -Fe<sub>2</sub>O<sub>3</sub> on a conducting FTO coated glass plate;
- Depositing RRPHTh-ND on a silicon or a conducting FTO coated glass plate; and
- Sandwiching the plate from (a) and the plate from (b) with polyvinyl alcohol (PVA)-hydrochloric acid based gel.

The disclosed RRPHTh-ND electrodes may provide high-sufficiency photoelectrochemical conversion an order of magnitude superior to existing TiO<sub>2</sub>-RRPHTh and ZnO-RRPHTh nanohybrid films.

In certain embodiments, the disclosed photoelectrochemical cells include MoS<sub>2</sub>- $\alpha$ -Fe<sub>2</sub>O<sub>3</sub> as a counter electrode and RRPHTh-ND as a working electrode. With MoS<sub>2</sub>- $\alpha$ -Fe<sub>2</sub>O<sub>3</sub> as an n-type electrode and RRPHTh-ND as a p-type electrode, the photoelectrochemical cells may further include a polyvinyl alcohol based gel as a solid electrolyte. In some embodiments, cyclic voltammetry (CV) and chronoamperometry experiments may be performed with visible light simulated for solar radiation and suitable radiation (e.g. 60 W lamp visible light radiation) to determine the photoelectrochemical properties of the disclosed cells.

In some embodiments, the disclosed solid gel based p-n photoelectrochemical cell according may show 100 order magnitude of photocurrent at different applied potentials.

Additionally, the disclosed p-n photoelectrochemical cell may be a stable solid state photoelectrochemical cell, which may greatly reduce any photocorrosion, preventing the leakage of solvent. It may also have low absorption of light due to a thin layer of electrolyte.

## 3. FURTHER ADVANTAGES

MoS<sub>2</sub> may play an important role for the charge transfer process with slow recombination of electron-hole pairs created due to photo-energy and having the charge transfer rate between surface and electrons.

A particularly advantageous configuration may be of an electrode including Fe<sub>2</sub>O<sub>3</sub>—MoS<sub>2</sub> and ND-RRPHTh as electrodes in a photoelectrochemical cell. MoS<sub>2</sub>- $\alpha$ -Fe<sub>2</sub>O<sub>3</sub> may be used as a cathode and ND-RRPHTh as an anode in a water based electrolyte including NaOH, HCl, H<sub>2</sub>SO<sub>4</sub>, acetic acid, etc.

Excellent photocurrent may be achieved using  $\alpha$ -Fe<sub>2</sub>O<sub>3</sub>—MoS<sub>2</sub>ND-RRPHTh as electrodes in photoelectrochemical cells or a photovoltaic device using a-hematite Fe<sub>2</sub>O<sub>3</sub>—MoS<sub>2</sub>/polyvinyl alcohol-HCl-ammonium sulphate (APS)/ND-RRPHTh.

The disclosed photoelectrochemical cells may be essentially free of any silicide material. The electrodes may also be essentially free of phosphate, carbonate, arsenate, phosphite, silicate, and/or borate.

MoS<sub>2</sub> particles may promote the electron transport properties of  $\alpha$ -Fe<sub>2</sub>O<sub>3</sub> nanomaterial by doping, homogenous structure, and dependability. The doping of MoS<sub>2</sub> particles may vary, for example, from about 0.1%, 0.2%, 0.5%, 1%, 2% to 5% in  $\alpha$ -Fe<sub>2</sub>O<sub>3</sub>. The  $\alpha$ -Fe<sub>2</sub>O<sub>3</sub> and MoS<sub>2</sub>- $\alpha$ -Fe<sub>2</sub>O<sub>3</sub> nanomaterials may be characterized by X-beam diffraction, SEM, FTIR, Raman spectroscopy, particle analysis, and UV-vis spectroscopy.

A nanodiamond blend with a conducting polymer as a p-type electrode in combination with  $\alpha$ -Fe<sub>2</sub>O<sub>3</sub> may be particularly advantageous.

A metal dichalcogenide may be selected, for example, from MoS<sub>2</sub>- $\alpha$ -Fe<sub>2</sub>O<sub>3</sub>, tungsten disulfide (WS<sub>2</sub>)- $\alpha$ -Fe<sub>2</sub>O<sub>3</sub>, molybdenum diselenide (MoSe<sub>2</sub>)- $\alpha$ -Fe<sub>2</sub>O<sub>3</sub>, molybdenum telluride- $\alpha$ -Fe<sub>2</sub>O<sub>3</sub>, tungsten selenide (WSe<sub>2</sub>), etc.

A gel electrolyte based on polymer and acid may be selected, for example, from polyvinyl alcohol, poly(vinyl acetate), poly(vinyl alcohol co-vinyl acetate), poly(methyl methacrylate), poly(vinyl alcohol-co-ethylene ethylene), poly(vinyl butyral-co-vinyl alcohol-co-vinyl acetate), poly-

vinyl butyral, polyvinyl chloride, and polystyrene. The combination of each polymer at different proportions can also be used for making the layer.

Further, the optical range may be increased by using  $TiO_2$ - $\alpha$ - $Fe_2O_3$  nanostructured film as n-type electrode.

There may be a ten to hundred fold of photo-current p-n junction based in such photoelectrochemical cell for water splitting application.

The photocurrent may be obtained at potential from about 0 to 2,000 V in p-n configuration of electrochemical cell.

As disclosed herein,  $\alpha$ - $Fe_2O_3$ - $MoS_2$  electrode was synthesized, and two orders of magnitude of photoelectrochemical properties was measured and 1%  $MoS_2$ - $\alpha$ - $Fe_2O_3$  shows the stable and nearly two orders of magnitude of stable photocurrent.

The photoelectrochemical photocurrent may be dependent on the concentration of the electrolyte.

One percent  $MoS_2$ - $\alpha$ - $Fe_2O_3$  deposited on a conducting ITO glass plate and RRPHTH-ND deposited on silicon or conducting FTO glass plates were sandwiched using polyvinyl alcohol (PVA)-hydrochloric acid based gel to fabricate solid gel based photoelectrochemical cell.

The p-n photoelectrochemical cell shows stable solid state photoelectrochemical cell and eliminates the photocorrosion process, prevents the leakage of solvent, and has low absorption of light due to thin layer of electrolyte.

The disclosed photoelectrochemical cells may be essentially free of sensitizers.

### 3. EXAMPLES

As non-limiting examples of the present technology, disclosed herein are photoelectrochemical cells having  $MoS_2$ - $\alpha$ - $Fe_2O_3$  as an n-type electrode and regioregular polyhexylthiophene-nanodiamond (RRPHTH-ND) as a p-type electrode. The photoelectrochemical cells may be liquid based or solid based.

#### Example 1

##### Molybdenum Disulfide Alpha-Hematite Nanocomposite Films

The nonmetal  $MoS_2$  is classified as a two-dimensional (2D) dichalcogenide material with a band gap of about 1.8 eV. It exhibits interesting photocatalytic activity, possibly due to its bonding, chemical composition, doping, and nanoparticle growth on various matrix films, and may also play an important role in charge transfer. As disclosed herein,  $MoS_2$  particles may be used to promote electron

nanomaterials. The doping of  $MoS_2$  particles varied by 0.1%, 0.2%, 0.5%, 1%, 2% and 5% in  $\alpha$ - $Fe_2O_3$ . The  $MoS_2$ - $\alpha$ - $Fe_2O_3$  nanomaterials were characterized using X-ray diffraction, SEM, FTIR, Raman spectroscopy, particle analyzer, and UV-vis techniques. Cyclic voltammetry (CV) and impedance measurements were utilized to understand the electrochemical electrode/electrolyte interface and photoelectrochemical properties of  $MoS_2$ - $\alpha$ - $Fe_2O_3$  based nanostructures for water splitting applications.

#### 10 Materials

The materials of iron chloride ( $FeCl_3$ ), aluminum chloride ( $AlCl_3$ ), sodium hydroxide ( $NaOH$ ),  $MoS_2$ , and ammonium hydroxide  $NH_4OH$  were purchased from commercial sources (Sigma-Aldrich). The fluorine tin oxide (FTO) coated glass with resistance of about  $10 \Omega/cm^2$  was also procured from commercial sources (Sigma-Aldrich). The centrifuged containers were purchased to clean the synthesized nanomaterials from the solution.

#### Experimental Procedure

$\alpha$ - $Fe_2O_3$  and  $MoS_2$ - $\alpha$ - $Fe_2O_3$  were synthesized by a sol-gel technique as shown in Eq.1. Table 1 shows the amount of chemicals used for the synthesis of  $MoS_2$ - $\alpha$ - $Fe_2O_3$ . Different concentrations of  $FeCl_3$  with  $AlCl_3$  were prepared in 500 ml round bottom flasks.  $NaOH$  solution was added to the resulting solution and stirred with a magnet for about an hour. A condenser was connected to the round bottom flask, which allowed the chemical reaction to proceed at about 90-100 °C. The reaction was terminated after about 24 hours, and the solution was cooled at about room temperature. The synthesized material was separated using a centrifuge and continuous cleaning with water. The synthesized materials ( $\alpha$ - $Fe_2O_3$  and  $MoS_2$ - $\alpha$ - $Fe_2O_3$ ) were initially left drying at about room temperature. FIG. 1 shows photographs of the materials synthesized using various percentages of  $MoS_2$  to  $\alpha$ - $Fe_2O_3$ . The immediate doping, such as 0.1%  $MoS_2$  changes the color of  $\alpha$ - $Fe_2O_3$ , whereas the dark red color can be visualized with the increase of  $MoS_2$  percentage in  $\alpha$ - $Fe_2O_3$ . The  $\alpha$ - $Fe_2O_3$  and  $MoS_2$ - $\alpha$ - $Fe_2O_3$  were dried at various temperatures (about 100, 200, 300, 400 and 500 °C.). In each case, the temperature was maintained in a furnace for about one hour. The materials were collected by cooling at room temperature and kept in a tight bottle for characterization as well as preparation of electrodes for electrochemical and photochemical tests.



TABLE 1

| Chemicals         | The amount of chemical used for synthesis of $MoS_2$ -composite $\alpha$ -hematite. |                                 |                                 |                               |                               |                               |
|-------------------|-------------------------------------------------------------------------------------|---------------------------------|---------------------------------|-------------------------------|-------------------------------|-------------------------------|
|                   | 0.1% $MoS_2$<br>w.r.t. $FeCl_3$                                                     | 0.2% $MoS_2$<br>w.r.t. $FeCl_3$ | 0.5% $MoS_2$<br>w.r.t. $FeCl_3$ | 1% $MoS_2$<br>w.r.t. $FeCl_3$ | 2% $MoS_2$<br>w.r.t. $FeCl_3$ | 5% $MoS_2$<br>w.r.t. $FeCl_3$ |
| $FeCl_3$          | 6.8 g                                                                               | 6.8 g                           | 6.8 g                           | 6.8 g                         | 6.8 g                         | 6.8 g                         |
| $MoS_2$           | 0.013 g                                                                             | 0.026 g                         | 0.065 g                         | 0.1296 g                      | 0.2592 g                      | 0.648 g                       |
| $NaOH$            | 4.8 g                                                                               | 4.8 g                           | 4.8 g                           | 4.8 g                         | 4.8 g                         | 4.8 g                         |
| $C_{19}H_{42}BrN$ | 0.5 g                                                                               | 0.5 g                           | 0.5 g                           | 0.5 g                         | 0.5 g                         | 0.5 g                         |

transport properties of  $\alpha$ - $Fe_2O_3$  nanomaterial by doping, homogenous structure, and dependability.

Under this work,  $MoS_2$  particles were used to promote electron transport properties of the  $\alpha$ - $Fe_2O_3$  nanomaterial by doping and homogenous structure due to  $MoS_2$ - $\alpha$ - $Fe_2O_3$

#### Film Formation of the Substrate

The  $MoS_2$ - $\alpha$ - $Fe_2O_3$  was prepared at different concentrations by mixing with acetic acid to obtain a homogenous solution to cast film on various substrates. About 500 mg of  $MoS_2$ - $\alpha$ - $Fe_2O_3$  (about 0.1%, 0.2%, 0.5%, 1%, 2%, and 5%)

was grinded and then mixed into about 10 ml acetic acid in a small container, and left for about 10 hours. Later, the colloidal solution containing  $\text{MoS}_2$ - $\alpha$ - $\text{Fe}_2\text{O}_3$  with acetic acid were used to make films on quartz, silicon, and fluorine tin oxide (FTO) coated glass plates. FIG. 1 shows the chemical structure of  $\text{MoS}_2$ - $\alpha$ - $\text{Fe}_2\text{O}_3$  nanomaterial (right) and photographs of synthesized  $\text{MoS}_2$ - $\alpha$ - $\text{Fe}_2\text{O}_3$  using different ratios of  $\text{MoS}_2$  to  $\text{Fe}_2\text{O}_3$ , such as about 0.1%, 0.2%, 0.5%, 1%, 2%, and 5%.

The films were cured at different temperatures (about 100, 200, 300, 400 and 500 °C.) for about one hour. The XRD, SEM, cyclic voltammetry, and UV-vis characterizations were performed in room temperature cooled  $\text{MoS}_2$ - $\alpha$ - $\text{Fe}_2\text{O}_3$  films. It has been observed that the nanomaterials treated at 100° C. to 200° C. could still have the water molecules. However, the temperature at around 300° C. allowed to have a solid material. The nanomaterials were further treated to 400° C. and 500° C. In some experiments, passivation, change in structure and morphology were observed in the samples treated at 300° C., 400° C. and 500° C. However, the results are presented for the samples treated at 500° C. due to their enhanced photocurrent.

#### UV-Vis Tests

FIG. 2 shows UV-vis spectra of  $\alpha$ - $\text{Fe}_2\text{O}_3$ ,  $\text{MoS}_2$  and  $\alpha$ - $\text{Fe}_2\text{O}_3$ - $\text{MoS}_2$ -prepared at a different ratio of  $\text{MoS}_2$  to  $\alpha$ - $\text{Fe}_2\text{O}_3$ . An UV-vis Spectrometer Jasco V-530 was used to measure the absorption spectra on various samples deposited on glass plates. FIG. 2A shows the UV-vis absorption at about 550 nm for pristine  $\alpha$ - $\text{Fe}_2\text{O}_3$ , as known in the art. FIG. 2B shows the characteristics absorption bands of about 388, 453, 618, and 679 nm for the  $\text{MoS}_2$  nanomaterial film on glass plates. FIGS. 2C-2F show the UV-vis absorption spectra for  $\text{MoS}_2$  doped in different percentages (about 0.1%, 0.2%, 1%, and 5%) with  $\alpha$ - $\text{Fe}_2\text{O}_3$  nanomaterial. FIG. 2C shows the absorption bands at about 282, 454, and 463 nm. FIG. 2D shows the absorption bands at about 446 and 565 nm. The distinct peaks can be seen at about 382, 461, and 570 nm. FIG. 2E shows the UV-vis bands at about 382, 456, and 559 nm, whereas FIG. 2F shows the absorption bands at about 382, 459, and 572 nm. There is a blue shift with an increase of  $\text{MoS}_2$  in a-hematite. However, the band observed for 0.1%  $\text{MoS}_2$  doping is shifted at about 572 nm in 5%  $\text{MoS}_2$  doping in  $\alpha$ - $\text{Fe}_2\text{O}_3$  nanomaterial. Such a result is consistent with the results shown for transition composite metal ions. The UV-vis spectra of the composite hematite have been estimated to be about 2.17 eV for the band at about 572 nm.

#### XRD Tests

The crystalline structure of  $\text{MoS}_2$ - $\alpha$ - $\text{Fe}_2\text{O}_3$ -nanocomposite was investigated by using Powder X-ray diffraction (XRD), model PANalytical X'Pert Pro MRD system with  $\text{Cu K}\alpha$  radiation (wavelength=1.5442 Å) operated at 40 kV and 40 mA. FIG. 3 shows X-ray diffraction curves for different percentages of  $\text{MoS}_2$  (about 0.1%, 0.2%, 0.5%, 1%, 2%, and 5%) to  $\alpha$ - $\text{Fe}_2\text{O}_3$ .  $\alpha$ - $\text{Fe}_2\text{O}_3$  has a polycrystalline structure as known from the XRD pattern. The diffraction common peaks of  $\text{MoS}_2$ - $\alpha$ - $\text{Fe}_2\text{O}_3$  nanocomposite with different percentages of  $\text{MoS}_2$  shows at 31.2°, 33.2°, 37.5°, 40.9°, 49.5°, 54.1°, 62.2°, and 64.2°, which can be indexed to (012), (104), (110), (113), (024), (116), (214), and (300) crystal planes of hexagonal iron oxide. It is clear from strong and sharp diffraction peaks that  $\alpha$ - $\text{Fe}_2\text{O}_3$  is well crystallized in the synthesis process for all percentage of  $\text{MoS}_2$  in  $\alpha$ - $\text{Fe}_2\text{O}_3$ . The peak at 54.1° may be due to the presence of  $\text{MoS}_2$  in the structure in  $\text{MoS}_2$ - $\alpha$ - $\text{Fe}_2\text{O}_3$ -nanocomposite.

#### FTIR Studies

A Perkin Elmer spectrum one was utilized to study FTIR spectroscopy of various samples of  $\text{MoS}_2$ - $\alpha$ - $\text{Fe}_2\text{O}_3$ -nanocomposite. The  $\text{MoS}_2$ - $\alpha$ - $\text{Fe}_2\text{O}_3$ -nanocomposite was mixed with KBr, the pellets were made using the hydraulic press, and the samples were measured using the transmission mode from 400 to 4000  $\text{cm}^{-1}$ . FTIR spectra of  $\text{MoS}_2$ - $\alpha$ - $\text{Fe}_2\text{O}_3$  shows the change of percentage of  $\text{MoS}_2$  doping with  $\alpha$ - $\text{Fe}_2\text{O}_3$  with Curve 1% to 5%, Curve 2% to 0.2%, Curve 3% to 2%, Curve 4 to 1%, Curve 5% to 0.5%, and Curve 6% to 0.1% of  $\text{MoS}_2$  in  $\text{MoS}_2$ - $\alpha$ - $\text{Fe}_2\text{O}_3$  in shown in FIG. 4. The infrared bands of each  $\text{MoS}_2$  doping to  $\alpha$ - $\text{Fe}_2\text{O}_3$  are shown in Table 2.

TABLE 2

| The Infrared bands of each $\text{MoS}_2$ doping to $\alpha$ - $\text{Fe}_2\text{O}_3$ . |                                                                   |
|------------------------------------------------------------------------------------------|-------------------------------------------------------------------|
| $\text{MoS}_2$                                                                           | Wavenumber ( $\text{cm}^{-1}$ )                                   |
| 5%                                                                                       | 474, 562, 620, 1136, 1193, 1472, 1642, 2858, 2924, 3436           |
| 2%                                                                                       | 484, 562, 620, 1136, 1193, 1472, 1642, 2858, 2924, 3436           |
| 1%                                                                                       | 474, 570, 640, 1006, 1134, 1388, 1470, 1670, 2854, 2924, 3436     |
| 0.5%                                                                                     | 458, 554, 644, 802, 898, 1042, 1386, 1468, 1634, 2856, 2922, 3438 |
| 0.1%                                                                                     | 512, 522, 654, 802, 1114, 1396, 1434, 1666, 2836, 2952, 3448      |

The hydroxyl (OH) group in  $\alpha$ - $\text{Fe}_2\text{O}_3$  is related to infrared band at 3414  $\text{cm}^{-1}$ . The band at 1642  $\text{cm}^{-1}$  is due to  $\nu$  (OH) stretching. The band at 562  $\text{cm}^{-1}$  is due to Fe—O vibration mode in  $\text{Fe}_2\text{O}_3$ . The band at 620-654 and 474-512 are related to the lattice defects in  $\text{Fe}_2\text{O}_3$ . The infrared band at 474-512  $\text{cm}^{-1}$  is due to stretching vibration depicting the presence of  $\text{MoS}_2$  in the  $\text{MoS}_2$ - $\alpha$ - $\text{Fe}_2\text{O}_3$  structure. The doping of 0.1% to 5% of  $\text{MoS}_2$  shifts the infrared band from 512  $\text{cm}^{-1}$  to 474  $\text{cm}^{-1}$ . The band at 474  $\text{cm}^{-1}$  is the band observed for exfoliated  $\text{MoS}_2$  nanosheets revealing that maximum doping in  $\text{MoS}_2$ - $\alpha$ - $\text{Fe}_2\text{O}_3$  structure.

#### SEM Tests

The scanning electron microscopy (SEM) of various  $\text{MoS}_2$ - $\alpha$ - $\text{Fe}_2\text{O}_3$  samples were measured using FE-SEM, S-800, Hitachi. FIG. 5 shows SEM images of  $\text{MoS}_2$ - $\alpha$ - $\text{Fe}_2\text{O}_3$  nanomaterials, which comprised different percentages, from 0.1% to 5%  $\text{MoS}_2$  to  $\text{Fe}_2\text{O}_3$  in  $\text{MoS}_2$ - $\alpha$ - $\text{Fe}_2\text{O}_3$ . SEM images show morphology of blooming flower-like nanoparticles with  $\text{MoS}_2$  doping in  $\text{MoS}_2$ - $\alpha$ - $\text{Fe}_2\text{O}_3$  for  $\text{MoS}_2$ - $\alpha$ - $\text{Fe}_2\text{O}_3$  structure. The images reveal that the size of the particle changes for the increase of  $\text{MoS}_2$  doping from 0.1% to 5% in  $\text{MoS}_2$ - $\alpha$ - $\text{Fe}_2\text{O}_3$  nanomaterial. It is difficult to recognize simple  $\alpha$ - $\text{Fe}_2\text{O}_3$  nanoparticles from  $\text{MoS}_2$  nanosheets, meaning a strong interface formation between  $\alpha$ - $\text{Fe}_2\text{O}_3$  and  $\text{MoS}_2$  in  $\text{MoS}_2$ - $\alpha$ - $\text{Fe}_2\text{O}_3$  nanomaterial.

#### Raman Spectroscopy

The Raman spectrum is measured which is also a rapid and nondestructive surface characterization technique to probe the vibrational properties of bonding of  $\text{MoS}_2$  to  $\text{Fe}_2\text{O}_3$  in  $\text{MoS}_2$ - $\alpha$ - $\text{Fe}_2\text{O}_3$  nanomaterial. FIGS. 6A and 6B show the Raman spectra of  $\text{MoS}_2$ - $\alpha$ - $\text{Fe}_2\text{O}_3$  film excited by 532 nm laser. The Raman shift at 532  $\text{cm}^{-1}$  resonates with the electronic transition in ring structures for aromatic clustering processes in  $\text{sp}^2$ -dominated particles. The shift associated at 374 and 417  $\text{cm}^{-1}$  are due to in-plane vibrational ( $\text{E}_{2g1}$ ) and the out-of-plane vibrational ( $\text{A}_{1g}$ ) modes. The enhanced  $\text{MoS}_2$  is indicative of energy difference between Raman shifts due to  $\text{MoS}_2$  content in  $\text{MoS}_2$ - $\alpha$ - $\text{Fe}_2\text{O}_3$  nanomaterial.

## Particle Analysis

The Zetasizer Nano particle analyzer range model was used to measure the average particle size of various  $\text{MoS}_2$ - $\alpha$ - $\text{Fe}_2\text{O}_3$  samples. Initially, the  $\text{MoS}_2$ - $\alpha$ - $\text{Fe}_2\text{O}_3$  nanomaterial was dispersed in water and ultra-sonicated to have aggregated free colloidal sample. FIG. 7 shows the particle size of  $\text{MoS}_2$ - $\alpha$ - $\text{Fe}_2\text{O}_3$  as a function of  $\text{MoS}_2$  doping in  $\alpha$ - $\text{Fe}_2\text{O}_3$ . The average particle size in liquid sample ranges from 459 nm (0.1%) to 825 nm for (5%) dopant of  $\text{MoS}_2$  respectively. Although these particles are small, there are few particles which are larger than 5 microns. These larger particles that can be detected through SEM measurement are a result of aggregation. The average size of particles is important for the fabrication of the electrodes from the particles. This information of nanomaterial dispersion of  $\text{MoS}_2$ - $\alpha$ - $\text{Fe}_2\text{O}_3$  can be exploited for the electrode fabrication or other applications.

## Cyclic Voltammetry

The electrochemical measurements on various  $\text{MoS}_2$ - $\alpha$ - $\text{Fe}_2\text{O}_3$  electrodes were measured from electrochemical workstation (Volta lab). The electrochemical set-up was adopted similar to earlier studies on hybrid films. FIG. 8 shows the cyclic voltammetry (CV) of 1%  $\text{MoS}_2$ - $\alpha$ - $\text{Fe}_2\text{O}_3$  in about 1 M NaOH as a working electrode, platinum (Pt) as a reference, and Ag/AgCl as reference electrode in three electrode based electrochemical cells. The continuous increase of CV current is observed with an increase in function of scan rate. The presence of  $\text{MoS}_2$  ions induces the electrochemical properties and about 1.3V can be seen as the oxidation potential of water, which is less than the Al-doped material.

The CV is shown in FIG. 9 with application of light simulated for solar radiation. However, at the scan rate of about 100 mV/sec, there is a maximum photocurrent absorbed for  $\text{MoS}_2$ - $\alpha$ - $\text{Fe}_2\text{O}_3$  film. The diffusion coefficient has been calculated using peak current for a reversible cyclic voltammetry is given by the Randles-Sevcik equation (Eq. 2). The diffusion coefficient has been estimated to be  $0.24 \times 10^{-16} \text{ cm}^2/\text{sec}$ .

$$I_p = (2.69 \times 10^5) n^{3/2} A C D^{1/2} v^{1/2} \quad \text{Eq. 2}$$

where  $I_p$  is current,  $n$  is number of electrons,  $A$  is electrode area ( $\text{cm}^2$ ),  $C$  is concentration ( $\text{mol}/\text{cm}^3$ ),  $D$  is diffusion coefficient ( $\text{cm}^2/\text{s}$ ), and  $v$  is potential scan rate (V/s).

## Chronoamperometry Tests

In some studies,  $\text{MoS}_2$ - $\alpha$ - $\text{Fe}_2\text{O}_3$  film was deposited on ITO coated glass substrates uniformly using the homogeneous paste obtained using acetic acid. The thickness of  $\text{MoS}_2$ - $\alpha$ - $\text{Fe}_2\text{O}_3$  was around 30  $\mu\text{m}$ . FIGS. 10A and 10B show the chronoamperometry tests of two electrodes cell consisting of  $\text{MoS}_2$ - $\alpha$ - $\text{Fe}_2\text{O}_3$  film as working and steel as counter in various concentrations (about 0.01, 0.1, and 1 M) of NaOH based electrolyte. The potential from about -1,000 mV to about 1,500 mV was applied, and the chronoamperometry photocurrent was studied. FIGS. 10A and 10B show the chronoamperometry photocurrent plot with  $t^{-1/2}$  for oxidation and reduction processes for  $\text{MoS}_2$ - $\alpha$ - $\text{Fe}_2\text{O}_3$  film. The rise of photocurrent shows  $t^{-1/2}$  linear with excitation of light. The current transient is different from the excitation of light. The diffusion-controlled photocurrent is calculated using the Cottrell equation in Eq. 3.

$$i = [nFAD^{1/2}C]/[\pi t^{1/2}] \quad \text{Eq. 3}$$

where  $n$  is the electron participating in the reaction,  $F$  is the faraday constant,  $A$  is the area of the electrode,  $i$  is the

transient current,  $D$  is the diffusion coefficient, and  $C$  is the concentration of the electrolyte.  $D$  was estimated to be  $1.057 \times 10^{-14} \text{ cm}^2/\text{sec}$ .

## Impedance Study

FIGS. 11A and 11B show the Nyquist plot in 1 M NaOH without and with light irradiation in  $\text{MoS}_2$ - $\alpha$ - $\text{Fe}_2\text{O}_3$  film in a photoelectrochemical set-up. The change in the impedance value has been observed for real and imaginary without light irradiation as shown in FIGS. 11A and 11B. The photocurrent is able to make process more conducting in presence of light.

## Half Sweep Potential

FIG. 10 shows the half sweep potential with and without light for both Al doped- $\alpha$ - $\text{Fe}_2\text{O}_3$  and  $\text{MoS}_2$ - $\alpha$ - $\text{Fe}_2\text{O}_3$ . Aluminum doping has shown the photocurrent to 35  $\mu\text{A}$  whereas for the same type of electrode for  $\text{MoS}_2$ - $\alpha$ - $\text{Fe}_2\text{O}_3$  shows the current till 150  $\mu\text{A}$ . Besides Schottky type current-voltage is experienced for both aluminum doped as well as  $\text{MoS}_2$ - $\alpha$ - $\text{Fe}_2\text{O}_3$  based electrode in photoelectrochemical cell.

Schematic of  $\text{MoS}_2$ - $\alpha$ - $\text{Fe}_2\text{O}_3$  Reaction Process

A schematic was drawn to understand the effect of  $\text{MoS}_2$  with  $\alpha$ - $\text{Fe}_2\text{O}_3$ . The schematic of hydrogen production using  $\text{MoS}_2$ -composite  $\alpha$ - $\text{Fe}_2\text{O}_3$  photocatalyst in about 1 M NaOH is shown in FIG. 13. The band gap of  $\text{MoS}_2$  varied from about 1.2-1.9 eV, whereas the band gap of  $\text{Fe}_2\text{O}_3$  is about 2.1 eV. The estimated band gap of  $\text{MoS}_2$ -composite  $\alpha$ - $\text{Fe}_2\text{O}_3$  in range of about 1.94 to 2.40 eV based on UV-vis measurements, which is well in the region of visible light.  $\text{MoS}_2$  doping also increases the conductivity of the samples. The schematic in FIG. 13 shows the photogenerated electrons from conduction band of  $\text{MoS}_2$  is transferred to conduction band (CB) of hematite whereas holes from hematite are transferred to valence band (VB) of  $\text{MoS}_2$ . This may enhance the photocatalytic activity of  $\text{MoS}_2$  composite with  $\text{Fe}_2\text{O}_3$  in  $\text{MoS}_2$ - $\alpha$ - $\text{Fe}_2\text{O}_3$  nanomaterial based electrode.

Thus, the synthesized  $\text{MoS}_2$ - $\alpha$ - $\text{Fe}_2\text{O}_3$  observed the shift in the band gap to 2.17 eV with  $\text{MoS}_2$  doping. There is a marked change in the band due to  $\text{MoS}_2$  doping in  $\alpha$ - $\text{Fe}_2\text{O}_3$ . The increase of  $\text{MoS}_2$  dominated the structure as marked from SEM measurements. The photocurrent can be clearly distinguishable with and without light irradiation through various electrochemical studies on  $\text{MoS}_2$ - $\alpha$ - $\text{Fe}_2\text{O}_3$  nanomaterial. The enhanced photocurrent is observed with  $\text{MoS}_2$  doping in  $\text{MoS}_2$ - $\alpha$ - $\text{Fe}_2\text{O}_3$  nanomaterial. The  $\text{MoS}_2$ - $\alpha$ - $\text{Fe}_2\text{O}_3$  nanomaterial thin film has the potential to produce hydrogen using a PEC water splitting process that could have renewable energy applications. These results may enable the use of  $\text{MoS}_2$ - $\alpha$ - $\text{Fe}_2\text{O}_3$  as n-type in p-n photoelectrochemical studies for efficient water splitting applications.

## Example 2

p-n Photoelectrochemical Cell Using  
 $\alpha$ -Hematite-Molybdenum Disulfide as n-Electrode  
 and Polyhexylthiophene (RRPHTh)—Nanodiamond  
 (ND) as P-Electrode

The recent momentum in energy research has simplified converting solar to electrical energy through photoelectrochemical (PEC) cells which can be closely compared to p-n junction solar cells. The PEC cells have numerous benefits, such as the inexpensive fabrication of thin film, reduction in absorption losses, due to transparent electrolyte, and a substantial increase in the energy conversion efficiency compared to the p-n junction based solar cells. Enhanced photocatalytic activity has been shown using molybdenum disulfide ( $\text{MoS}_2$ ) doped alpha ( $\alpha$ )-hematite ( $\text{Fe}_2\text{O}_3$ ) over

$\alpha$ -Fe<sub>2</sub>O<sub>3</sub> nanomaterials, due to the materials its bonding, chemical composition, doping and nanoparticles growth on the graphene films. The photoelectrochemical properties of p-n junction of PEC cell using polyhexylthiophene (RRPHTh) conducting polymer and nanodiamond (ND) as p-type and MoS<sub>2</sub>- $\alpha$ -Fe<sub>2</sub>O<sub>3</sub> nanocomposite films as n-type electrode materials were explored.

The  $\alpha$ -Fe<sub>2</sub>O<sub>3</sub>-MoS<sub>2</sub> nanocomposite material was synthesized using sol-gel technique, and characterized using SEM, X-ray diffraction, UV-vis, FTIR and Raman techniques, respectively. The other electrode nanomaterial as ND-RRPHTh was synthesized using reported method (Ram et al., The Journal of Physical Chemistry C, 2011. 115(44): p. 21987-21995). The electrochemical techniques were utilized to understand the photocurrent, electrode and the electrolyte interface of  $\alpha$ -Fe<sub>2</sub>O<sub>3</sub>-MoS<sub>2</sub> and ND-RRPHTh nanocomposite films. The photoelectrochemical properties of p-n junction of MoS<sub>2</sub>- $\alpha$ -Fe<sub>2</sub>O<sub>3</sub>-ND-RRPHTh, deposited on either n-type silicon or FTO-coated glass plates, showed 3-4 times higher in current density and energy conversion efficiencies than parent electrode materials in an electrolyte of 1M of NaOH in PEC cells. Nanomaterials based electrode  $\alpha$ -Fe<sub>2</sub>O<sub>3</sub>-MoS<sub>2</sub> and ND-RRPHTh have shown an improved hydrogen release compared to  $\alpha$ -Fe<sub>2</sub>O<sub>3</sub>, aluminum  $\alpha$ -Fe<sub>2</sub>O<sub>3</sub> and MoS<sub>2</sub> doped  $\alpha$ -Fe<sub>2</sub>O<sub>3</sub> nanostructured films in PEC cells.

Nano-hybrid RRPHTh with various dopant (TiO<sub>2</sub>, ZnO, and nanodiamond) has previously been used for photoelectrochemical applications. RRPHTh-nanodiamond (ND) electrode has been used to provide high-sufficiency photoelectrochemical conversions superior to TiO<sub>2</sub>-RRPHTh and ZnO-RRPHTh nanohybrid film (U.S. Pat. No. U.S. 9,416,456, which is incorporated herein by reference). Here, the use of MoS<sub>2</sub>- $\alpha$ -Fe<sub>2</sub>O<sub>3</sub> as n-electrode and RRPHTh-ND as p-electrode in liquid-based photoelectrochemical cells was studied in PEC cells. MoS<sub>2</sub>- $\alpha$ -Fe<sub>2</sub>O<sub>3</sub>, as counter electrode, and RRPHTh-ND, as a working electrode, were used to study the photoelectrochemical cells. The CV, chronoamperometry studies were performed with visible light, radiation simulated for solar radiation as well as with 60 W lamps, to understand the photoelectrochemical properties of PEC cells.

#### Materials

The materials iron chloride (FeCl<sub>3</sub>), aluminum chloride (AlCl<sub>3</sub>), sodium hydroxide (NaOH), MoS<sub>2</sub>, poly(3-Hexylthiophene) and ammonium hydroxide (NH<sub>4</sub>OH) were purchased from Sigma-Aldrich. The fluorine tin oxide (FTO) coated glass, with resistance of  $\sim$ 10 $\Omega$ , was also procured from Sigma-Aldrich. The centrifuged containers were purchased to clean the synthesized nanomaterials from the solution.

#### Synthesis of Nanomaterials

The  $\alpha$ -Fe<sub>2</sub>O<sub>3</sub> and MoS<sub>2</sub>- $\alpha$ -Fe<sub>2</sub>O<sub>3</sub> were synthesized by a sol-gel technique. Different concentrations of FeCl<sub>3</sub> with AlCl<sub>3</sub> were prepared in 500 ml round bottom flasks. Later, NaOH was added to the resulting solution and stirred with a magnet. A condenser was connected to the round bottom flask, containing the chemicals, then placed in a heater to maintain 90-100° C. for the chemical reaction. The reaction was terminated after 24 hours, and the solution was cooled at room temperature. The synthesized material was separated using a centrifuge and continuous cleaning with water. The synthesized materials (MoS<sub>2</sub>- $\alpha$ -Fe<sub>2</sub>O<sub>3</sub>) were initially left drying at room temperature. The MoS<sub>2</sub>- $\alpha$ -Fe<sub>2</sub>O<sub>3</sub> was then dried at various temperatures (100, 200, 300, 400 and 500° C.). In each case, the temperature was maintained in a furnace for one hour. The materials were then brought to

room temperature, and collected in a tight bottle for photoelectrochemical and various physical characterization studies.

#### Film Formation of Substrate

The MoS<sub>2</sub>- $\alpha$ -Fe<sub>2</sub>O<sub>3</sub> was prepared at different concentrations by mixing it with acetic acid to obtain a homogenous solution to cast on various substrates. 500 mg of MoS<sub>2</sub>- $\alpha$ -Fe<sub>2</sub>O<sub>3</sub> (0.1%, 0.2%, 0.5%, 1%, 2% and 5%) was ground into a powder and then mixed into 10 ml acetic acid in a small 10 container and left for 10 hours. Later, the solutions were used to make films on quartz, silicon and fluorine tin oxide (FTO). The films were cured at different temperatures (300, 400 and 500° C.) for one hour. The films were cooled to room temperature and used for XRD, SEM, cyclic voltammetry and UV-vis measurements.

#### RRPHTH-ND/NaOH/Fe<sub>2</sub>O<sub>3</sub>-ND Based Photoelectrochemical Cell

The conducting polymer solution was made by dissolving about 50 mg of RRPHTh in about 50 ml of chloroform. 20 Later, about 50 mg of nanodiamond (ND) was added to the solution and kept stirring for about 24 hours. The RRPHTh-ND film was fabricated using spin coating as well as by casting the solution on silicon and ITO coated glass substrates. The photoelectrochemical cell was constructed using silicon as well as ITO coated RRPHTh-ND as the working electrode and MoS<sub>2</sub>- $\alpha$ -Fe<sub>2</sub>O<sub>3</sub> as the counter electrode. The cyclic voltammetry (CV) as well as the chronoamperometry measurements were made using 0.1 M and 1M NaOH concentration. FIG. 23A shows the schematic of hydrogen production using MoS<sub>2</sub>-composite  $\alpha$ -Fe<sub>2</sub>O<sub>3</sub> photocatalyst in 1 M NaOH based electrolyte in a PEC cell.

#### SEM

The structure and surface properties of  $\alpha$ -Fe<sub>2</sub>O<sub>3</sub>, MoS<sub>2</sub>- $\alpha$ -Fe<sub>2</sub>O<sub>3</sub> and RRPHTh+ND films on silicon substrates were 35 investigated through Field Emission Hitachi 5800 Scanning Electron Microscope (SEM) with EDS attachment which, worked at 25 kV. FIG. 14A shows SEM image of  $\alpha$ -Fe<sub>2</sub>O<sub>3</sub> nanomaterial consisting of well-dispersed spheres with particle sizes of 100-300 nm. The particle sizes have increased 40 in MoS<sub>2</sub>- $\alpha$ -Fe<sub>2</sub>O<sub>3</sub> (FIG. 14B). The films consisting of  $\alpha$ -Fe<sub>2</sub>O<sub>3</sub>, as well as MoS<sub>2</sub>- $\alpha$ -Fe<sub>2</sub>O<sub>3</sub> have uniform and dense spheres of particles. The ND hybrid with RRPHTh conducting polymer has particle sizes varying from 100 nm to 500 nm. The average size of nanoparticles of ND was kept at around 20 nm. The RRPHTh provides a nearly uniform 45 covering over the ND particles forming the nano-hybrid structure.

#### FTIR

The infrared bands at 467 and 523 cm<sup>-1</sup> are related to 50 Fe—O stretching and bending vibration mode for  $\alpha$ -Fe<sub>2</sub>O<sub>3</sub> nanomaterial as shown in FIG. 15A. FIG. 15B shows FTIR spectra of  $\alpha$ -Fe<sub>2</sub>O<sub>3</sub>+0.1% MoS<sub>2</sub>. It shows IR bands at 1388 and 1407 cm<sup>-1</sup> which are related to the stretching vibration as well as in-plane bending vibration of O—H of  $\alpha$ -Fe<sub>2</sub>O<sub>3</sub> 55 nanomaterial. Moreover, the IR bands at 544 and 1630 cm<sup>-1</sup> are assigned to O—H<sup>+</sup> group which is in-plane bending vibration and  $\gamma_{as}$  Mo—S vibration that is due to the presence of MoS<sub>2</sub>. However, the bands at 638, 802, and 892 are generated due to out of plane bending vibration and  $\gamma_{as}$  60 Mo—O vibrations, which is related to OH<sup>+</sup> group. In addition, Fe—O presence shows stretching vibration in  $\alpha$ -Fe<sub>2</sub>O<sub>3</sub>+0.1% MoS<sub>2</sub>. FIG. 15C shows FTIR spectra of RRPHTh+ND, and various bands are also presented in Table 3. The bands at 1739 cm<sup>-1</sup> is the characteristics 65 band of nanodiamond, the presence of 1687, 1129 and 630 cm<sup>-1</sup> are due to the presence of functional group in the nanodiamond . The RRPHTh characteristics peaks (413,

475, 514, 758, 800, 852, 1000, 1058, 1092, 1260, 1300, 1390, 1446, 1497, 1635, 1687, and 1820) are shown in FIG. 15C which can be well compared with the work of Ram et al.

TABLE 3

The infrared bands of each  $\alpha$ -Fe<sub>2</sub>O<sub>3</sub>, 0.1% MoS<sub>2</sub>, RRPHTh + ND.

| Material                                 | Infrared bands in $\text{cm}^{-1}$                                                                                           |
|------------------------------------------|------------------------------------------------------------------------------------------------------------------------------|
| $\alpha$ -Fe <sub>2</sub> O <sub>3</sub> | 467, 523, 578, 796, 830, 872, 990, 1046, 1076, 1376, 1551, 1625, 1736, 1763                                                  |
| 0.1% MoS <sub>2</sub>                    | 512, 522, 654, 802, 1114, 1396, 1434, 1666, 2836, 2952, 3448                                                                 |
| RRPHTh + ND                              | 413, 475, 514, 630, 758, 800, 852, 1000, 1058, 1092, 1129, 1260, 1300, 1390, 1446, 1497, 1635, 1687, 1739, 1820, 2089, 3415, |

#### XRD

The model PAN-alytical X'Pert Pro MRD system operated at 40 kV and 40 mA was used to measure X-ray diffraction having CuK $\alpha$  radiation of wavelength=1.5442 Å. FIG. 16A shows XRD image of  $\alpha$ -Fe<sub>2</sub>O<sub>3</sub> nanomaterial. The  $\alpha$ -Fe<sub>2</sub>O<sub>3</sub> nanomaterial reveals a polycrystalline structure and coincides with the values as earlier investigated by Hussein et al. Table 4 shows the summary of diffraction angle 2theta angles. FIG. 16B shows the sharp diffraction angle of XRD spectra of  $\alpha$ -Fe<sub>2</sub>O<sub>3</sub>+0.1% MoS<sub>2</sub>. The sharp diffraction angle peak at 31.69 (012), 36.62 (110), 45.46 (024), 53.23 (116), 58.93 (214) are due to the crystallinity of Fe<sub>2</sub>O<sub>3</sub> as well as the presence of doping of MoS<sub>2</sub> in  $\alpha$ -Fe<sub>2</sub>O<sub>3</sub>+0.1% MoS<sub>2</sub> nanomaterial. However, the band at 53.23 is related to MoS<sub>2</sub> in MoS<sub>2</sub>- $\alpha$ -Fe<sub>2</sub>O<sub>3</sub> nanomaterial.

TABLE 4

The diffraction common peaks of each  $\alpha$ -Fe<sub>2</sub>O<sub>3</sub>, Fe<sub>2</sub>O<sub>3</sub> + 0.1% MoS<sub>2</sub>, RRPHTh + ND

|                                |                                                                              |
|--------------------------------|------------------------------------------------------------------------------|
| Fe <sub>2</sub> O <sub>3</sub> | 30.41, 32.11, 33.87, 39.83, 44.68, 45.54, 47.76, 63.89, 66.16, 72.96, 76.085 |
| 0.1% MoS <sub>2</sub>          | 31.69, 36.62, 45.46, 53.23, 58.93                                            |

#### UV-Vis

An UV-Vis spectrometer Jasco V-530 was utilized to determine the absorption peaks of different nanomaterials such as  $\alpha$ -Fe<sub>2</sub>O<sub>3</sub>,  $\alpha$ -Fe<sub>2</sub>O<sub>3</sub>+0.1% MoS<sub>2</sub>, and RRPHTh+ND (Table 5). FIG. 17A shows UV-vis absorption spectra of  $\alpha$ -Fe<sub>2</sub>O<sub>3</sub> film on ITO coated glass plate. The absorption band at 550 nm was depicted similar to the previous study by Hussein et al (Surface Review and Letters, 2017: p. 1950031). The characteristics absorption bands at 373, 382, 406, 442, 475, 612 nm of  $\alpha$ -Fe<sub>2</sub>O<sub>3</sub>+0.1% MoS<sub>2</sub> were observed in FIG. 17B. FIG. 17C reveals the characteristics bands at 412, 475, 503, 588, 695, 834 nm for ND+RRPHTH based film similar to the previous work by Ram et al. (American Journal of Analytical Chemistry, 2017. 8(08): p. 523). The band gap of MoS<sub>2</sub> varies from 1.2-1.9 eV, whereas the band gap of  $\alpha$ -Fe<sub>2</sub>O<sub>3</sub> is 2.1 eV. So, the band gap of MoS<sub>2</sub>-composite  $\alpha$ -Fe<sub>2</sub>O<sub>3</sub> was estimated to be in the range of 1.94 to 2.4 eV, which is well fit in the region of visible light. MoS<sub>2</sub> doping increases the conductivity of the samples. The schematic in FIG. 18 shows photogenerated electrons from conduction band (CB) of MoS<sub>2</sub> that gets transferred to CB of hematite whereas holes from hematite are transferred to valance band (VB) of MoS<sub>2</sub>. This doping enhances the photocatalytic activity of MoS<sub>2</sub> composite with  $\alpha$ -Fe<sub>2</sub>O<sub>3</sub>.

TABLE 3

| The UV-vis absorption peaks of each $\alpha$ -Fe <sub>2</sub> O <sub>3</sub> , Fe <sub>2</sub> O <sub>3</sub> + 0.1% MoS <sub>2</sub> , RRPHTh + ND |                                                                        |                                                                                         |
|-----------------------------------------------------------------------------------------------------------------------------------------------------|------------------------------------------------------------------------|-----------------------------------------------------------------------------------------|
| 5                                                                                                                                                   | Fe <sub>2</sub> O <sub>3</sub><br>0.1% MoS <sub>2</sub><br>RRPHTh + ND | 286, 346, 371, 470, 580<br>373, 382, 406, 442, 475, 612<br>412, 475, 503, 588, 695, 834 |

Photo-Electrochemical Studies on p-n Junction Based on MoS<sub>2</sub>- $\alpha$ -Fe<sub>2</sub>O<sub>3</sub> and RRPHTh-ND Electrodes in Photoelectrochemical Cell

The MoS<sub>2</sub>- $\alpha$ -Fe<sub>2</sub>O<sub>3</sub> as n-electrode and RRPHTh-ND as p-electrode in liquid electrolyte (1M NaOH, HCl etc.) was studied in photoelectrochemical cells. In some studies, solid electrolyte (e.g. PVA-HCl or PVA-H<sub>3</sub>PO<sub>4</sub> gel) based photoelectrochemical cells were also tested. The cyclic voltammetry and the chronoamperometry studied on the p-n junction based photoelectrochemical cell with and without light extensively. FIG. 18 shows the water splitting application in RRPHTH-ND as p and MoS<sub>2</sub>-Fe<sub>2</sub>O<sub>3</sub> as n-type in 1M NaOH water-based electrolyte photoelectrochemical cell under a photoexcitation and applied electrical potential. The NaOH was used as electrolyte in the photoelectrochemical cell. The cyclic voltammetry (CV) as well as the chronoamperometry measurements were made using 0.1 M and 1M concentrations of NaOH based electrolytes.

Attempts were made to understand the water splitting using work function and band gap of the material. The MoS<sub>2</sub> doped  $\alpha$ -Fe<sub>2</sub>O<sub>3</sub> in water has band gap varying from 2.5 to 1.94 eV. The hydrogen gas was formed at electrode of RRPHTH-ND whereas oxygen was liberated at MoS<sub>2</sub>- $\alpha$ -Fe<sub>2</sub>O<sub>3</sub> based electrode.

#### Cyclic Voltammetry Study of MoS<sub>2</sub>- $\alpha$ -Fe<sub>2</sub>O<sub>3</sub> and RRPHTh-ND Electrodes in Photoelectrochemical Cell

FIG. 19 shows the cyclic voltammetry curves with and without light for MoS<sub>2</sub>- $\alpha$ -Fe<sub>2</sub>O<sub>3</sub> and RRPHTh-ND based electrodes in 0.1M NaOH solution. The CV curves show nearly twice the value of photocurrent than without light. However, at light under 2V shows exposition the photocurrent which varies 30 times greater current for n type based electrode containing 1% MoS<sub>2</sub> - $\alpha$ -Fe<sub>2</sub>O<sub>3</sub> in p-type RRPHTh-ND containing 1M NaOH electrolyte.

#### Chronoamperometry Study of MoS<sub>2</sub>- $\alpha$ -Fe<sub>2</sub>O<sub>3</sub> and RRPHTh-ND Electrodes in Photoelectrochemical Cell

FIG. 20 below shows the chronoamperometry curves of MoS<sub>2</sub>- $\alpha$ -Fe<sub>2</sub>O<sub>3</sub> and RRPHTh-ND in 0.1 M NaOH solution. The light bulb of 60 W was exposed and the immediate current in the device increased significantly for 0.1% MoS<sub>2</sub>- $\alpha$ -Fe<sub>2</sub>O<sub>3</sub> as n-type and RRPHTh-ND as p-type electrode in a cell containing 0.1M NaOH electrolyte. The photocurrent is observed with the exposure to light on the cell. However, the transient current was immediately observed due to the combination of electron and hole-pair, and there is a decrease of photocurrent in 0.1% MoS<sub>2</sub>- $\alpha$ -Fe<sub>2</sub>O<sub>3</sub> as n-type and RRPHTh-ND as p-type electrode based electrodes in photoelectrochemical cell.

FIG. 21 shows chronoamperometry results of 0.1, 0.2, 1, and 5% of MoS<sub>2</sub> in  $\alpha$ -Fe<sub>2</sub>O<sub>3</sub> MoS<sub>2</sub> as n-type electrode and RRPHTh-ND as p-type electrode in a cell containing 0.1M NaOH electrolyte. The current density was found to be highest for 1% MoS<sub>2</sub>- $\alpha$ -Fe<sub>2</sub>O<sub>3</sub> as n-type electrode with RRPHTh-ND as p-type electrode in a cell containing 0.1M NaOH electrolyte. There is a current transient but it becomes a stable photocurrent after 2-3 sec whereas there is continual decrease of photocurrent in 0.1 and 0.2% of MoS<sub>2</sub> in  $\alpha$ -Fe<sub>2</sub>O<sub>3</sub> nanocomposite material. However, 5% of MoS<sub>2</sub> in

$\alpha$ -Fe<sub>2</sub>O<sub>3</sub> nanocomposite material does not reveal higher photocurrent due to aggregation of MoS<sub>2</sub> in  $\alpha$ -Fe<sub>2</sub>O<sub>3</sub> nanomaterial.

FIG. 22 shows chronoamperometry results of 0.1, 0.2, 1, and 5% of MoS<sub>2</sub> in  $\alpha$ -Fe<sub>2</sub>O<sub>3</sub> MoS<sub>2</sub> as n-type electrode and RRPHTH-ND as p-type electrode in a cell containing 0.1M NaOH electrolyte at a potential of 2000 mV. The current density was found to be highest for 0.1 and 1% MoS<sub>2</sub>- $\alpha$ -Fe<sub>2</sub>O<sub>3</sub> based n-type based electrode. There was a larger current transient for 0.1% MoS<sub>2</sub> in MoS<sub>2</sub>- $\alpha$ -Fe<sub>2</sub>O<sub>3</sub> nanocomposite material. However, stable photocurrent after 2-3 sec was also observed for 1% of MoS<sub>2</sub> in MoS<sub>2</sub>- $\alpha$ -Fe<sub>2</sub>O<sub>3</sub> nanocomposite nanomaterial film. The chronoamperometry results revealed that 1% MoS<sub>2</sub> in MoS<sub>2</sub>- $\alpha$ -Fe<sub>2</sub>O<sub>3</sub> nanocomposite was a suitable structure to obtain higher photocurrent density.

#### Hydrogen Production

FIG. 23A shows the schematic of hydrogen production using MoS<sub>2</sub>-composite  $\alpha$ -Fe<sub>2</sub>O<sub>3</sub> photocatalyst in 1M NaOH based electrolyte in a PEC cell. FIG. 23B shows the chemical structure of nanodiamond in a regioregular polyhexylthiophene blend structure.

Thus, MoS<sub>2</sub>- $\alpha$ -Fe<sub>2</sub>O<sub>3</sub> electrodes were synthesized to measure their photoelectrochemical properties in the water splitting process. The films, for example consisting of  $\alpha$ -Fe<sub>2</sub>O<sub>3</sub> as well MoS<sub>2</sub>- $\alpha$ -Fe<sub>2</sub>O<sub>3</sub>, have a uniform and dense sphere of particles. The 1% MoS<sub>2</sub>- $\alpha$ -Fe<sub>2</sub>O<sub>3</sub> film showed the most stable photocurrent. From the XRD figure, the band at 53.23 is related to MoS<sub>2</sub> in MoS<sub>2</sub>- $\alpha$ -Fe<sub>2</sub>O<sub>3</sub> nanomaterial. The photoelectrochemical photocurrent was found to be dependent on the applied potential, from 0 to 2V, in an electrolyte of varying molar concentration of NaOH. The chronoamperometry results showed that 1% MoS<sub>2</sub> in MoS<sub>2</sub>- $\alpha$ -Fe<sub>2</sub>O<sub>3</sub> nanocomposite may be a suitable structure to obtain a higher photocurrent density. The p-n photoelectrochemical cell may be a stable photoelectrochemical cell and allows for eliminating the photo corrosion process. Also, this p-n junction may prevent the leakage of solvent and may have low absorption of light, due to the thin layer of electrolytes. The disclosed materials may provide a renewable and affordable process to produce clean energy in the form of hydrogen. Accordingly, PEC with 1% MoS<sub>2</sub>- $\alpha$ -Fe<sub>2</sub>O<sub>3</sub> nanocomposite has a great potential for application in fuel cell technology.

#### Example 3

##### Solid Photoelectrochemical Cell

The photocurrent is studied for the solid photoelectrochemical cell based on RRPHTH-ND as p-electrode and MoS<sub>2</sub>-Fe<sub>2</sub>O<sub>3</sub> or TiO<sub>2</sub>-Fe<sub>2</sub>O<sub>3</sub> as n-electrode in PVA-HCl based electrolyte. FIG. 24 shows the schematic of solid photoelectrochemical cell electrolyte. The n-type electrode “MoS<sub>2</sub>-Fe<sub>2</sub>O<sub>3</sub>” is shown in FIG. 24. However, other n-type electrode Fe<sub>2</sub>O<sub>3</sub>-TiO<sub>2</sub>, Fe<sub>2</sub>O<sub>3</sub>-zinc oxide (ZnO), Fe<sub>2</sub>O<sub>3</sub>-tin oxide (SnO<sub>2</sub>), Fe<sub>2</sub>O<sub>3</sub>-tungsten oxide (WO<sub>3</sub>), Al<sub>2</sub>O<sub>3</sub>-Fe<sub>2</sub>O<sub>3</sub>, or combination can be chosen for the fabrication of solid photoelectrochemical cell.

FIG. 25 shows the chronoamperometry studies on photoelectrochemical cell consisting of RRPHTH-ND as p-electrode and MoS<sub>2</sub>-Fe<sub>2</sub>O<sub>3</sub> as n-electrode in PVA-HCl based electrolyte. FIG. 25 shows the current transient in photoelectrochemical cell from about 0 to 2,000 mV with light switch on and off condition. The about 60 watt lamp was used for the chronoamperometry study. Interestingly, at about 0 mV potential application reveals the current tran-

sient regardless of light switch on condition for nearly about 10 sec whereas there is minor current transient for the potential varying from about 500 mV to 2,000 mV for the light switch on condition.

5 The photoelectrochemical cell is also fabricated using the other n-type “0.05% TiO<sub>2</sub>-Fe<sub>2</sub>O<sub>3</sub>” and RRPHTH-ND as p-electrode in PVA-HCl gel based electrolyte. The current density is nearly a hundred times larger than the light switch on condition. The photocurrent has been obtained for each 10 potential from about 0 to 2,000 mV application to the cell (FIG. 26).

15 As disclosed herein,  $\alpha$ -Fe<sub>2</sub>O<sub>3</sub>-MoS<sub>2</sub> electrode was synthesized and the photoelectrochemical properties were measured. About 1% MoS<sub>2</sub>- $\alpha$ -Fe<sub>2</sub>O<sub>3</sub> shows the stable photocurrent. The photoelectrochemical photocurrent is dependent to the applied potential from about 0 to 2 V in an electrolyte of varying molar concentration of NaOH. The disclosure is also about the configuration of photoelectrochemical cell for hydrogen splitting through anode and cathode electrodes. 20 Later, about 1% MoS<sub>2</sub>- $\alpha$ -Fe<sub>2</sub>O<sub>3</sub> deposited on conducting ITO glass plate and RRPHTH-ND deposited on silicon or conducting FTO glass plates were sandwiched using polyvinyl alcohol (PVA)-hydrochloric acid based gel to fabricate solid gel based photoelectrochemical cell. The solid gel based p-n photoelectrochemical cell has been studied under about 60 watt and solar simulated light which shows the about 100 order magnitude of photocurrent at different applied potential. The p-n photoelectrochemical cell shows stable solid state photoelectrochemical cell and eliminates the photocorrosion process, prevents the leakage of solvent, and has low absorption of light due to thin layer of electrolyte.

25 Thus, the invention provides, among other things, a photoelectrochemical cell. Various features and advantages of the invention are set forth in the following claims.

What is claimed is:

1. A photoelectrochemical cell comprising:

(a) an n-type electrode comprising MoS<sub>2</sub>- $\alpha$ -Fe<sub>2</sub>O<sub>3</sub> nanocomposite film, wherein the MoS<sub>2</sub>- $\alpha$ -Fe<sub>2</sub>O<sub>3</sub> has an average particle size of from 459 nm to 825 nm;

(b) a p-type electrode comprising a conducting polymer, wherein the conducting polymer is polyhexylthiophene; and

(c) an electrolyte.

2. The photoelectrochemical cell of claim 1, wherein the MoS<sub>2</sub>- $\alpha$ -Fe<sub>2</sub>O<sub>3</sub> nanocomposite film comprises a dopant selected from the group consisting of platinum, tin, cobalt, zinc, palladium, titanium, chromium, rhodium, iridium, and combinations thereof.

3. The photoelectrochemical cell of claim 1, wherein the conducting polymer is regioregular polyhexylthiophene.

4. The photoelectrochemical cell of claim 1, wherein the p-type electrode comprises an electron acceptor selected 55 from the group consisting of diamond, nanodiamond, hexagonal boron-nitride (hBN), graphite, methyl [6, 6]-phenyl-C61-butylate (PCBM), 2,4,7-trinitro-9-fluorenone, copper-phthalocyanines, and combinations thereof.

5. The photoelectrochemical cell of claim 1, wherein the 60 electrolyte is an aqueous electrolyte comprising sodium hydroxide, potassium hydroxide, magnesium hydroxide, lithium hydroxide, sodium chloride, potassium chloride, magnesium chloride, hydrochloric acid, sulfuric acid, nitric acid, acetic acid, butyric acid, lactic acid, oxalic acid, myristic acid, and/or perchloric acid.

6. The photoelectrochemical cell of claim 1, wherein the 65 electrolyte is a gel comprising a polymer and an acid.

## 19

7. The photoelectrochemical cell of claim 6, wherein the polymer is selected from the group consisting of polyvinyl alcohol, poly(vinyl acetate), poly(vinyl alcohol co-vinyl acetate), poly(methyl methacrylate), poly(vinyl alcohol co-ethylene ethylene), poly(vinyl butyral co-vinyl alcohol co-vinyl acetate), polyvinyl butyral, polyvinyl chloride, poly-styrene, and combinations thereof.

8. The photoelectrochemical cell of claim 6, wherein the acid is selected from the group consisting of acetic acid, propionic acid, hydrochloric acid, hydrofluoric acid, phosphoric acid, sulfuric acid, formic acid, benzoic acid, hydrofluoric acid, nitric acid, phosphoric acid, sulfuric acid, tungstosilicic acid hydrate, hydriodic acid, carboxylic acid, and combinations thereof.

9. The photoelectrochemical cell of claim 1, wherein the nanocomposite film is deposited on a conducting fluorine tin oxide (FTO) coated glass plate.

10. The photoelectrochemical cell of claim 1, wherein the photoelectrochemical cell is capable of being stable, of being essentially free of photocorrosion, of preventing leakage of solvent, and/ or of having low absorption of light.

15

## 20

11. The photoelectrochemical cell of claim 1, wherein the intensity of a photocurrent produced by the photoelectrochemical cell is dependent on the concentration of the electrolyte.

12. The photoelectrochemical cell of claim 1, capable of at least a 100 times difference in stable photocurrent at different applied potentials.

13. The photoelectrochemical cell of claim 1, wherein the  $\text{MoS}_2\text{-}\alpha\text{-Fe}_2\text{O}_3$  nanocomposite film has from 0.1 wt % to 5 wt %  $\text{MoS}_2$ .

14. A method of generating hydrogen from water comprising:

(a) providing a photoelectrochemical cell according to claim 1; and

(b) splitting water into hydrogen and oxygen by a photocurrent produced by the photoelectrochemical cell.

15. The method of claim 14, wherein the photocurrent has a potential from about 0 V to about 2,000 V.

\* \* \* \* \*